

May 30, 1972

H. VAN DEN BERG ET AL

3,666,504

PROCESS FOR PREPARING MOULDING SAND

Filed March 29, 1971

3 Sheets-Sheet 1

FIG. 1



INVENTORS  
HENDRIK VANDEN BERG  
HERMAN G. LEVELINK  
BY  
Hammond and Weeks  
ATTORNEYS

May 30, 1972

H. VAN DEN BERG ET AL

3,666,504

PROCESS FOR PREPARING MOULDING SAND

Filed March 29, 1971

3 Sheets-Sheet 2

FIG. 2



INVENTORS  
HENDRIK VAN DEN BERG  
HERMAN G. LEVELINK  
BY

*Hendrik van den Berg*  
ATTORNEYS

May 30, 1972

H. VAN DEN BERG ET AL

3,666,504

PROCESS FOR PREPARING MOULDING SAND

Filed March 29, 1971

3 Sheets-Sheet 3

FIG. 3



INVENTORS  
HENDRIK VANDEN BERG  
HERMAN G. LEVELINK  
BY  
*Hendrik and J. G. Levelink*  
ATTORNEYS

1

3,666,504

**PROCESS FOR PREPARING MOULDING SAND**  
Hendrik van den Berg, 36 Isaac da Costalaan, Delft, Netherlands, and Herman G. Levelink, 34 Julianalaan, Pijnacker, Netherlands  
Continuation-in-part of abandoned application Ser. No. 867,612, Oct. 20, 1969. This application Mar. 29, 1971, Ser. No. 128,689  
Claims priority, application Netherlands, Oct. 22, 1968, 6815124  
Int. Cl. B28b 7/34  
U.S. Cl. 106—38.35 5 Claims

## ABSTRACT OF THE DISCLOSURE

A process is described for preparing a moulding sand having improved properties over ordinary moulding sand as for fluidity, moisture content, cohesion and scabbing resistance by adding to ordinary moulding sand a maximum of 2% by weight of pulverized cocoa beans or parts of them such as ground cocoa shells or cocoa expellers.

## PRIOR APPLICATION

This application is a continuation-in-part application of copending, commonly assigned U.S. patent application Ser. No. 867,612 filed Oct. 20, 1969, now abandoned.

## STATE OF THE ART

The invention relates to a process for preparing moulding sand.

The material for moulds used in the casting process mainly comprises sand with a binding agent. As a binding agent hereby as a rule clay is used. Such a type of sand is found in nature as a ready product or can be synthetically composed of quartz sand with a bentonite or another clay as binding agent.

Dependent on the nature of the castings the metal is cast into a wet or dried mould.

For iron castings some percents of powdered coal or pitch are added to the sand for wet moulds, to prevent that the moulding sand will adhere too strongly to the casting, while dried moulds for this purpose as a rule are provided with a coating.

The moulding sand must meet certain requirements connected with transport and storage and with the behaviour of this sand in the casting moulding proper.

In the moulding process a homogeneous ramming of the sand around the pattern must be obtained with a possibility of a good separation of mould and pattern and a casting product must be created which is free from surface defects and is an accurate copy of the pattern.

The extent to which a homogeneous ramming of the moulding sand can be achieved is strongly dependent upon the fluidity of the sand.

In case of insufficient fluidity of the moulding sand, in the mould alongside the walls of the pattern, less compacted spots are created which cause a casting with a rough surface.

The less compacted spots alongside the wall of the moulding box and in the corners of the moulding-box may give rise to mould-wall movements during or immediately after casting causing dimensional inaccuracy of the casting.

2

The fluidity of the sand is in fact determined by the tendency towards inter-grain cohesion of the sand.

As the tendency towards cohesion in the sand increases, already in filling the moulding-box, for instance, from a hopper this sand will show more coherence and even in this loose bulk condition less sand will reach the deeper lying and with difficulty accessible parts of the mould as a result of blocking.

Even the subsequent compacting operations are insufficient to eliminate this inhomogeneity.

So the fluidity of the moulding sand in loose bulk condition is an important property with respect to the workability of the sand and decisive for the final condition of the compacted mould.

Besides, the cohesion of the moulding sand in compacted condition is of importance.

It must be feasible to separate the mould from the pattern without mould pieces being broken off and remaining on the pattern.

This is particularly important with moulds that are lifted from the pattern by a tilting movement, which occurs fairly often in practice. The then permissible deformation of the sand can be measured by determining the so-called angle of tilting with the aid of a standard test piece. The angle of tilting thereby is the angle at which the moulding sand starts to crack.

The usefulness of clay-bonded moulding sand with respect to filling, compacting and stripping of the mould further is strongly dependent on the moisture content.

This moisture content may only vary within specific limits which limits may for instance be determined with the aid of the so-called Dietert mouldability-tester. Herewith a certain amount of sand is rotated in a drum-shaped screen for a certain time and at a certain speed. A certain percentage of the sand goes through the screen, depending on the moisture content and consequently on the tendency towards cohesion. This percentage is a measure for the "mouldability" of this sand, and as a rule moulding sand with a good workability has a mouldability from 70 to 90.

By casting metal into the mould, stresses may arise in the surface layer of the mould by a sudden heating of the moulding sand and attendant expansion. These stresses may be so great that this layer gets loose from the substrate and peeling occurs.

A peel thus formed may bend, break off, or be eroded causing various types of scab to be created in the surface of the casting.

The tendency of the moulding sand towards this peeling, the so-called "scabbing tendency," may also be determined experimentally by exposing a test piece to shock-heating.

In order to be able to meet in the foundry technique the demands that are becoming increasingly higher with respect to the above properties, it is known in the art to use certain additives for the moulding sand that have an advantageous effect on these properties.

It has been found that, for instance, cellulose products, such as wood flour, powdered flax seed-vessel, powdered wheat seed-vessel and the like reduce the scabbing tendency of clay-bonded moulding sand. The influence on the fluidity, however, is very slight and negative on the angle of tilting.

Besides, starch derivatives such as "cereals," dextrin and the like in case of this sand have an advantageous influence on the scabbing resistance and stripping prop-

erties of moulding sand, but the fluidity then strongly decreases.

Consequently disadvantages of these additives are that only certain properties of the moulding sand become more advantageous, other valuable properties on the other hand worsen.

### THE INVENTION

Surprisingly it has been found that a type of moulding sand can be prepared whereby the above disadvantages do not occur and whereby a moulding sand is obtained whose properties mentioned above meets the requirements without disadvantageous side-effects arising.

For his purpose, according to the invention, the process for preparing moulding sand from sand, one or more binding agents and other additives is characterized by the addition of between 0.05 to 2% by weight of cocoa beans powder.

By cocoa beans powder is meant a free flowing pulverized product from cocoa beans from which the greater part of cocoa butter has been removed.

Such products show varying fat contents of at most 15% by weight. An example of such powder products is the pulverized cocoa press cake.

However, since this product is used as cocoa powder in beverages, it is rather expensive for technical uses.

The defatted pulverized cocoa waste products which more advantageously can be applied in our invention are for instance; (a) the ground cocoa expeller cake (having an average fat content of 11% by weight); (b) the ground defatted or extracted cocoa expeller cake which is also called cocoa extracted meal powder; (c) the same product after the theobromine recovery process; and (d) the ground commercial cocoa shells (having an average fat content of about 3% by weight). Kirk-Othmer Encyclopedia of Chemical Technology, vol. 2, first edition, p. 890 and 891 illustrates how some of these products may be obtained, namely cocoa expeller cake and cocoa press cake.

According to the invention the cocoa beans powder may also be added to a moulding sand that is largely composed of return sand, but then added in very small quantities, partly because the return sand may already contain cocoa beans powder from a previous moulding sand preparation, partly because this return sand, to obtain one and the same advantageous effect, needs a slight addition, owing to the condition in which the binding agent of this sand is.

To moulding sand composed of new sand with a binding agent, in the process according to the invention preferably 0.1-1% by weight of ground extracted cocoa expeller cake is added.

The advantageous effects of the process for preparing moulding sand of the invention are further elucidated below with reference to some graphs and further herein-after some examples are given of moulding sand compositions with which these advantageous effects are obtained.

As additive to the moulding sand, ground extracted cocoa expeller cake is used.

In FIG. 1 the fluidity of the moulding sand in percentages as an ordinate at A is plotted against the moisture content in percentages as an abscis at B.

In this FIG. 1, curve I shows the moulding sand composed of quartz sand, 6% by weight of sodium bentonite and 4% by weight of powder coal, with an addition of 1/2% by weight of ground extracted cocoa expeller cake.

Curve I' shows this moulding sand with the same percentages of bentonite and powder coal, but in this case with an addition of 1/2% by weight of corncobs powder and curve II shows the moulding sand without addition.

In this comparative chart curve I clearly shows the improvement in fluidity of the moulding sand with the addition of ground extracted cocoa expeller cake as compared with the addition of corncobs powder (curve I').

In FIG. 2 the angle of tilting as ordinate at C is plotted against the moisture content as an abcis at B.

Here curve III shows the moulding sand with an addition of 2% by weight of ground extracted cocoa expeller cake, and curve III' gives as an addition the same percentage by weight of corncobs powder.

5 In this figure curve III gives a strong improvement of the angle of tilting as compared with the moulding sand without addition (see curve IV), and further from curve III' the negative influence of an addition of corncobs powder clearly emerges, this curve being even worse than the moulding sand without addition (curve IV).

10 Further in FIG. 3 the course of the moldability at D is indicated in dependence upon the moisture percentage at B.

15 From this figure it also appears clearly that the moulding sand with the addition of 1/2% by weight of ground extracted cocoa expeller cake (see curve V) is workable over a much wider moisture range than moulding sand without such an addition or with an equal addition of corncobs powder.

20 When casting into moulding sand with an addition of ground extracted cocoa expeller cake it was further found that this addition reduces the scabbing tendency to at least the same extent as when a good quality of cereals would be used.

25 Casting experiments have shown that by the improvement of the above properties of moulding sand by adding cocoa bean powder a more dimensionally accurate casting will be obtained.

30 By this addition the tendency towards inter-grain cohesion of the sand grains in the loose bulk condition and enveloped by clay is considerably lower. Thereby the transport of the moulding sand from the sand preparation plant to the sand hoppers can run more easily.

35 The flow of the sand from the hopper into the moulding box will also present fewer problems, since the sand has less tendency to "hang."

40 It is remarkable that the ground extracted cocoa expeller cake, also after extraction of, for instance, theobromine from it, as is applied in the chemical industry still has the same advantageous effect when added to moulding sand as untreated extracted cocoa expeller cake.

45 Examples of compositions from which clay-bonded moulding sand according to the invention has been prepared, are:

#### EXAMPLE I.—NEW SAND

100 parts by weight of quartz sand, 6% of bentonite, 3% of powdered coal, 1/2% of ground extracted cocoa expeller cake and water.

#### EXAMPLE II.—FACING SAND

70 parts by weight of return moulding sand, 30 parts by weight of quartz sand, 2.5% of bentonite, 1/2% of powdered coal, 0.2% of ground extracted cocoa expeller cake and water.

#### EXAMPLE III.—UNIT SAND

97 parts by weight of return moulding sand, 3 parts by weight of quartz sand, 0.3% of bentonite, 0.15% of powdered coal, 0.05% of ground extracted cocoa expeller cake and water. (Note: all percentages are by weight.)

60 In Examples No. II and III, by a repeated use of return sand, only a very small addition of ground extracted cocoa expeller cake is required to maintain the advantageous properties of the moulding sand.

65 Various modifications of the process and compositions of the invention may be made without departing from the spirit or scope thereof and it should be understood that the invention is to be limited only as defined in the appended claims.

70 We claim:

1. In the process for preparing a sand composition for foundry molds comprising mixing said with a clay binder, the improvement comprising adding to said composition 0.05 to 2.0% by weight of cocoa bean powder.

2. The process of claim 1 wherein the sand is new sand and the cocoa bean powder is ground extracted cocoa expeller cake.

3. The process of claim 2 wherein the said expeller cake is present in an amount of 0.1 to 1% by weight.

4. In a foundry moulding composition comprising sand and clay, the improvement comprising maintaining in said composition 0.05 to 2% by weight of cocoa bean powder.

5. A moulding composition of claim 4 wherein the said powder is 0.1 to 1.0% by weight of ground extracted cocoa expeller cake.

No references cited.

5 LORENZO B. HAYES, Primary Examiner

U.S. Cl. X.R.

106—38.5, 38.9, 68